

April 29, 1924.

1,492,230

W. M. TOWNE

PROCESS FOR WORKING ZINC

Filed Aug. 21, 1922

Fig. 1.



Fig. 3.



Fig. 4.



Fig. 5.



INVENTOR :  
Walter M. Towne,  
By Attorneys,

Fraser, Durk & Myers

## UNITED STATES PATENT OFFICE.

WALTER M. TOWNE, OF BROOKLYN, NEW YORK, ASSIGNEE, BY DIRECT AND MESNE ASSIGNMENTS, TO E. W. BLISS COMPANY, OF NEW YORK, N. Y., A CORPORATION OF NEW YORK.

## PROCESS FOR WORKING ZINC.

Application filed August 21, 1922. Serial No. 583,269.

To all whom it may concern:

Be it known that I, WALTER M. TOWNE, a citizen of the United States of America, residing in the borough of Brooklyn, county of Kings, city and State of New York, have invented certain new and useful Improvements in Processes for Working Zinc, of which the following is a specification.

This invention relates to a method of making zinc tubular articles, especially those in the form of cups or containers. The invention provides means for forming such articles by extrusion.

Heretofore such articles of zinc have been most commonly made by forming sections of tube and soldering to one end of each a disk. This is a difficult soldering operation, and the articles thus made are unduly expensive.

Another method which has been successfully practised consists in cutting a blank from sheet zinc and drawing it into cup form between dies, the diameter being reduced in successive stages, and the cup elongated to bring it to the required size and shape. For a cylindrical cup with a length about twice its diameter, usually four successive drawing operations are required, necessitating four sets of dies and a corresponding number of re-handlings of the articles in course of production. The present invention enables such cup-shaped articles to be produced with one pair of dies and at one stroke.

According to the present invention, a suitably shaped blank is first formed of a diameter not exceeding that of the cup to be made, and of such thickness as to afford the requisite amount of metal. This blank is of soft zinc of suitable purity and homogeneity. It is placed in the cavity of a die or matrix having parallel outer surfaces corresponding in diameter and outline to the exterior dimensions of the cup or article to be formed. A male die or punch is provided of corresponding but smaller outline, the difference in size agreeing with the desired thickness of the walls of the cup to be made. This punch being properly guided and centered is forced downward into the matrix under suitable pressure, whereby the blank being squeezed between the dies is caused to flow out or extrude through the

annular space between them, so that the walls of the cup being formed flow up along the punch, this operation being continued with the descent of the punch until the cup reaches the proper dimensions; that is to say, until the end of the punch approaches as closely to the bottom of the cavity in the matrix as is desired to give the bottom of the cup the proper thickness. The active portion of the punch is at its lower end where the metal flows from its bottom around its sides, and directly above this active portion the punch is reduced or tapered back, so as to relieve the flowing zinc of internal pressure and friction immediately after its extrusion. The operation is performed with the zinc at a temperature closely approximating 150° C.

The accompanying drawings illustrate one embodiment of the invention, comprising dies for forming a cup-shaped article or cylindrical container.

Figure 1 is a vertical mid-section of the male die or punch.

Fig. 2 is a similar section of the female die or matrix.

Fig. 3 is an oblique elevation of the blank.

Fig. 4 is a sectional view, showing the condition during the early part of the extruding operation.

Fig. 5 is a similar view, the punch being in elevation, showing the completion of the operation.

Referring to the drawings, A is the punch or male die and B the female die or matrix. The latter is formed with a cavity or hollow b, which in plan is of the shape and dimensions of the exterior of the article to be formed (being circular for a cylindrical article), and having a depth somewhat more than sufficient to receive the thickness of the blank shown in Fig. 3. This thickness will vary for a given diameter with the variations in the length of the article to be made and in the thickness of its walls. The inner walls of the matrix are formed perpendicular to the plane of the die, that is parallel with the relative direction of movement of the dies during extrusion. The bottom of the matrix is curved, flat or otherwise according to the shape to be given to the bottom of the article to be formed. The

punch A is of a length somewhat exceeding that of the article to be formed, and of a diameter corresponding therewith; its lower outer portion *a*, being the active portion 5 around which the zinc flows during extrusion, is shaped in plan according to the contour and size of the interior of the article to be formed; in case the article has walls of uniform thickness, the bottom portion *a* has 10 the same contour in plan as the recess *b* except that it is sufficiently smaller to allow for the thickness of the walls. The bottom *c* of the punch is made flat or curved according to the shape of the interior of the 15 bottom of the cup or other article to be formed. If this bottom portion is to be of uniform thickness, the bottom *c* of the punch is made parallel with the bottom of the cavity in the matrix or die B. The punch is 20 reduced in diameter directly above the active portion *a* by being tapered back so as to relieve the zinc of pressure as soon as the flowing zinc has been conformed between the portions *a* *b* of the dies. The punch A is 25 provided with a shank portion A' of any suitable shape and construction to fit the corresponding member of the press in which the dies are to be used. In a press of the usual construction the die B will be carried 30 in a die block on the bed of the press and the punch A will have its shank A' centered and fastened in a bolster or other fitting fastened to the moving head or platen of the press. Usually the construction of such 35 presses is sufficiently close and accurate to guide the punch and die in proper relation and keep the punch properly centered with reference to the cavity in the die. In Fig. 1 the punch is shown as having within it a 40 knock-out bar D enlarged at its lower end to form a head *d* which constitutes a portion of the bottom *c* of the punch. The bar D projects out through the top of the punch to a suitable height so that its upper end may be 45 struck by a stop or operating lever in the manner well understood in presses of this kind. Preferably the knock-out bar is held up by a spring *e* pressing upwardly against a collar *f*.

50 In practising the process of this invention, it is desirable for the most successful results to conform to the following requirements:

55 The blank is to be made of soft zinc of such approximation to purity as will cause it to flow uniformly. Zinc having a scleroscopic (Shore test) hardness of not over 23 should be used in order that the proper working condition may be obtained through 60 subjection to heat for a short time. The zinc should have a lead content not exceeding 0.6 per cent and a cadmium content not exceeding 0.5 per cent. It is preferable to use pack rolled zinc by reason of its more favorable property as to grain due to roll-

ing. Pack rolled zinc gives better results than strip-rolled zinc, which has a decided grain and has been found to be more ductile in direction with the grain than across the grain. For this reason when strip rolled 70 zinc is used, the extruded cup runs high on diametrically opposite sides where the flow is with the grain and low on the other two sides where the flow is across the grain, so that the extrusion leaves the metal under 75 unequal strain and more scrap has to be trimmed off, and it is more difficult to control the height of the extruded cup. The use of pack rolled zinc avoids these disadvantages, since it has a substantial absence 80 of grain direction, and the extrusion affords substantially uniform strain around the cup and runs to a uniform height.

It is important that the zinc be worked at a temperature approximating as closely as 85 possible to 150° C. This temperature gives sufficient plasticity and ductility to form a cup or tube with a thin wall. For thicker walls or purer zinc a lower temperature is 90 admissible; but the method finds its most 95 advantageous use in making cups with thin walls, and using zinc with approximately the percentage of lead and cadmium above indicated. At lower temperatures the internal friction of the metal increases, and it 98 becomes stiffer and more difficult to extrude. At higher temperatures there is a decrease in its ductility. In practice the blank should be heated to a somewhat higher temperature 100 to make allowance for the cooling of the blank while being placed in the dies and for the heat taken up by the dies. The precise drop to be thus allowed for must be determined in each case by experiment.

105 The proper lubrication of the blank is practically important. The best lubricant thus far found is lard oil. Only sufficient lubricant should be used to form a very thin film on the blank; if more is applied, it is desirable to rub off the excess so as to 110 leave the blank apparently clean. An excess of lubricant causes the metal to rupture in the forming of the cup or tube, and introduces difficulty in controlling the flow of the metal. If no lubricant or insufficient lubricant be used, the zinc is liable to flake in the dies, and the latter are subjected to excessive wear.

115 The final essential to successful extrusion is the exercise of precision in the reciprocal 120 formation of the die surfaces and the extreme hardening of these surfaces. It has been found that zinc can be successfully extruded only when the dies are so conformed 125 that an equal and uniform flow of the metal occurs from the beginning of the pressure to the finish of the extruding stroke. If because of faulty construction or conformation of the dies, the metal is allowed to become pocketed or retarded at any point, so 130

that its flow is not thus continuous, it will immediately stiffen and lose its plasticity. For this reason the described construction of the active faces of the die cavity and the 6 punch, or some other conformation for obtaining the same result, must be provided. The lower outer edge *a* of the punch around which the extruding metal flows in beginning its ascent along the outer wall of the 10 die cavity should be formed with a sharply rounded corner. Directly above this corner the metal should be tapered back, so as to relieve its pressure against the inner face of the extruding metal so that the latter may 15 flow as freely as possible after having been shaped between the die surfaces, and whereby needless friction and consequent waste of power are avoided. For clearness this tapering back or reduction of the punch is some- 20 what exaggerated in Figs. 4 and 5. It is to be understood that the diminution does not need to be sufficient to bring the outer face of the punch actually out of contact with the inner face of the flowing wall of 25 metal, but need be only enough to diminish frictional adhesion, the amount of which in the drawing would be nearly imperceptible. The lower outer corner of the bottom of the die cavity should be very slightly rounded, 30 being made as sharp as is mechanically possible.

It is important to have a suitable conformation between the bottom *c* of the punch and the bottom of the die cavity, in order 35 not only to give the desired shape to the bottom of the cup to be formed, but what is more important, to cause the extruding metal to flow uniformly from the center outwardly to the annular space between the 40 punch and matrix. The flow should be slowest at the center and should accelerate uniformly in radial lines toward the outer wall, the maximum rate of flow being through the contracted annular space where the extrusion finally occurs.

Owing to the tendency of the zinc to hug or close in around the punch, it has been found advisable to remove the cup after extrusion by the action of an ejector or knock-out, such as that shown at D.

The dies having been properly formed, it is important that their surfaces be rendered extremely hard. I have found that a scleroscopic hardness (Shore test) of 90 or upward gives practically successful results.

The present invention provides a method by which a more homogeneous and perfect cup of zinc can be produced than by the previous methods. Such cups are largely used as the zinc element in a dry battery, and for this purpose it is important that the molecular structure of the zinc be as uniform as possible. The drawing method heretofore used has required for its success 65 a zinc of exceptional purity in its freedom

from lead, cadmium, etc. and consequently a very expensive form of zinc. The drawn zinc battery shell has also been defective by reason of the difference in crystalline structure set up in its walls by the multiplicity 70 of drawing operations; thus each time the shell is reduced in diameter by drawing, the effect is to create a zone extending around the shell having a smaller grain structure than the metal intervening between that 75 zone and the one created by the next subsequent reducing operation. This condition causes a variation in the susceptibility of the metal to corrosion through contact with the chemicals of the battery. This disadvantage is wholly avoided by the present invention, which produces drawn cups or shells in a single operation, and with walls of uniform crystalline structure.

The extruding operation leaves the cup 85 with a slightly irregular upper edge and the extruded cups are afterward trimmed to a uniform height, as shown for example by the line *x*—*x* in Fig. 5.

What I claim is:—

1. The process of working zinc which consists in subjecting a blank to pressure between male and female dies and extruding it through a contracted annular space surrounding the male die in a direction opposite to the movement of the male die, and while at a temperature approximating 150 degrees C.

2. The process of claim 1, the blank being of soft zinc practically free from grain formation.

3. The process of claim 1, the blank being of zinc having a lead content not exceeding 0.6 per cent.

4. The process of claim 1, the blank being of zinc having a cadmium content not exceeding 0.5 per cent.

5. The process of claim 1, the blank being of zinc having a lead content not exceeding 0.6 per cent and a cadmium content not exceeding 0.5 per cent.

6. The process of working zinc, which consists in subjecting a blank to pressure within the cavity of a female die by forcing thereinto a male die of smaller diameter, 115 and extruding it through an annular space between such dies in a direction opposite to the movement of the male die, and while at a temperature approximating 150 degrees C.

7. The process of working zinc which consists in subjecting a blank to pressure within the cavity of a female die by forcing thereinto a male die, having its largest diameter at its bottom portion, between which and the inner wall of the female die the zinc 125 is extruded, and the male die diminished in diameter immediately above such bottom portion to relieve the extruded metal of pressure.

8. The process of working zinc which 130

consists in subjecting a blank to pressure within the cavity of a female die by forcing thereinto a male die, having its largest diameter at its bottom portion, between which and the inner wall of the female die the zinc is extruded, and the male die at its end conformed to the contour of the bottom of the

cavity in the female die, and both relatively shaped to impart a continuous outward flow to the metal between them during extrusion. 10

In witness whereof, I have hereunto signed my name.

WALTER M. TOWNE.